

UNITED STATES PATENT OFFICE.

WILHELM BERN, OF LUDWIGSHAFEN, GERMANY, ASSIGNOR TO BADISCHE  
ANILIN & SODA FABRIK, OF LUDWIGSHAFEN, GERMANY, A CORPORA-  
TION OF BADEN.

## PROCESS OF DISCHARGING INDIGO-DYED WOOL.

**SPECIFICATION** forming part of Letters Patent No. 690,847, dated December 31, 1901.

Application filed January 23, 1901. Serial No. 44,455. (No specimens.)

*To all whom it may concern:*

Be it known that I, WILHELM BERNs, doctor of philosophy and chemist, a subject of the King of Prussia, German Emperor, residing at Ludwigshafen-on-the-Rhine, in the Kingdom of Bavaria, Germany, have invented new and useful Improvements in Processes of Discharging Indigo-Dyed Wool, of which the following is a specification.

10 The processes for producing white or colored discharge effects on indigo-dyed wool at present known are, so far as I am aware, more or less unsatisfactory. For instance, by attempting to apply to wool the chromate 15 discharge process as used for indigo-dyed cotton it is found impossible to obtain even impure whites, as hardly any destruction of the indigo on the parts printed is effected, and the colored effects obtained by this method 20 are on this account insufficiently brilliant. I have found that by the addition of certain steps to the known discharging process exceedingly pure white and colored discharge effects on indigo-dyed wool can be produced; 25 and my invention consists in the addition of these steps to and in the combination of these steps with the known discharging process. The said steps are, first, steaming the goods after having printed them with a discharge 30 ing composition, and, second, treating the goods with a bleaching agent—such a sulfurous acid, hydrogen peroxid, potassium percarbonate, and the like after having discharged them.

35 The following examples will serve to further illustrate the nature of this invention and the manner of carrying it into practical effect; but the invention is not confined to the examples. The parts are by weight.

40 *Example 1—White discharge effect on indigo-dyed wool.*—Print indigo-dyed woolen material with a discharge composed of three hundred and fifty (350) parts of tragacanth-water, six (6) per cent.; four hundred (400) parts of gum-water (1:1); one hundred and twenty-five (125) parts of water, and three hundred (300) parts of sodium bichromate, (powder.) Steam the goods for five (5) min-

utes in a Mather-Platt apparatus and pass them for about twenty (20) seconds at a temperature of fifty-five (55) to fifty-seven (57) degrees centigrade through a bath containing fifty (50) grams of oxalic acid, fifty (50) grams of sulfuric acid (containing ninety-five (95) per cent.  $H_2SO_4$ ) in one (1) liter of solution, and then leave for several hours in a bleaching-bath made up of five hundred (500) parts of hydrogen peroxid, (containing about two (2) to three (3) per cent.  $H_2O_2$ ), five hundred (500) parts of water, and fifteen (15) parts of ammonia solution, (containing about twenty (20) per cent.  $NH_3$ .) Wash and dry. In place of hydrogen peroxid aqueous sulfurous acid, bisulfite-of-soda solution, gaseous sulfurous acid, or potassium percarbonate can be employed.

*Example 2—Red discharge effect on indigo-dyed wool.*—Print the indigo-dyed wool with a mixture of three hundred (300) parts tragacanth-water, six (6) per cent.; three hundred (300) parts of gum-water (1:1); six hundred and ten (610) parts of water, sixty (60) parts of indulin scarlet, and three hundred (300) parts of powdered sodium bichromate. Steam the goods. Pass them through the discharging-bath, as in Example 1, and bleach them with an alkaline solution of hydrogen peroxid or with aqueous sulfurous acid of four (4) degrees Baumé or with sodium-bisulfite solution of five (5) degrees Baumé, or with an atmosphere of gaseous sulfurous acid. 75 80

In place of indulin scarlet methylene blue B extra can be used to produce blue effects, azoflavin 3G. for greenish - yellow effects, azoflavin 3R. for reddish-yellow effects, and rhodamin extra for carmine effects, while of course, if desired, multicolored effects or colored effects in combination with white effects can be produced on the same goods. 85

Now what I claim is—

1. The process for producing discharge effects on indigo-dyed wool which consists in printing the goods with a discharging-paste, steaming them and bleaching them when discharged with a suitable bleaching agent, substantially as hereinbefore described. 95

2. The process for producing discharge effects on indigo-dyed wool which consists in printing the goods with a discharging-paste, containing a suitable coloring-matter, steaming them and bleaching them when discharged with a suitable bleaching agent, substantially  
5 as hereinbefore described.

In testimony whereof I have hereunto set my hand in the presence of two subscribing witnesses.

WILHELM BERN.

Witnesses:

OSCAR BALLY,  
JOHN L. HEINKE.